

[54] SILVER HALIDE PHOTOGRAPHIC EMULSION SENSITIZED WITH A HETEROCYCLIC COMPOUND CONTAINING 4-SULFUR ATOMS

[75] Inventors: Reiichi Ohi; Mitsunori Sugiyama; Yosuke Nakajima; Michio Horie, all of Ashigara; Shigeru Kobayashi, Osaka, all of Japan

[73] Assignee: Fuji Photo Film Co., Ltd., Ashigara-Kamigun, Kanagawa, Japan

[22] Filed: Oct. 16, 1973

[21] Appl. No.: 406,991

**Related U.S. Application Data**

[63] Continuation-in-part of Ser. No. 210,568, Dec. 21, 1971, abandoned.

[30] **Foreign Application Priority Data**

Dec. 21, 1970 Japan ..... 45-114544

[52] U.S. Cl. ..... 96/107, 96/108

[51] Int. Cl. ..... G03c 1/28

[58] Field of Search ..... 96/107, 108

[56] **References Cited**

UNITED STATES PATENTS

3,622,329 11/1971 Huchstadt et al. ..... 96/107

3,656,955 4/1972 Ushimaru et al. ..... 96/107

Primary Examiner—Norman G. Torchin

Assistant Examiner—Won H. Louie, Jr.

Attorney, Agent, or Firm—Sughrue, Rothwell, Mion, Zinn & Macpeak

[57] **ABSTRACT**

A novel sensitizer for silver halide photographic emulsions represented by the formula:



where  $R_1$ ,  $R_2$ ,  $R_3$  and  $R_4$  individually represent hydrogen atoms or alkyl or aralkyl groups, and  $R_1$  and  $R_3$  may combine, respectively, with  $R_2$   $R_4$  to form cycloalkyl groups.

The sensitizing effect of the sensitizer compound can be improved by using the compound in combination with a compound which will liberate a thiosulfate ion, without increasing fog formation.

20 Claims, 3 Drawing Figures





FIG. 1

FIG. 2  
(pH7)FIG. 3  
(pH9)

**SILVER HALIDE PHOTOGRAPHIC EMULSION  
SENSITIZED WITH A HETERO CYCLIC  
COMPOUND CONTAINING 4-SULFUR ATOMS**

**CROSS REFERENCE TO RELATED  
APPLICATIONS**

This application is a continuation-in-part application of copending application Ser. No. 210,568, filed Dec. 21, 1971, now abandoned based on Japanese application No. 114544/70, filed Dec. 21, 1970, the priority of which is claimed.

**BACKGROUND OF THE INVENTION**

**1. Field of the Invention**

This invention relates to a silver halide photographic emulsion and, in particular, to a silver halide photographic emulsion which has been chemically sensitized with a stable sulfur containing compound.

**2. Description of the Prior Art**

In the manufacture of photographic emulsion, many chemical sensitization processes are known for the enhancement of photographic sensitivity. For instance, compounds containing one or more unstable sulfur atoms in the molecule, such as, e.g., sodium thiosulfate and thiourea derivatives, are known sulfur sensitizers, and certain reducing agents, such as, e.g., stannous chloride and hydrazine, are known reductive sensitizers. Some of these unstable sulfur containing compounds and reductive compounds are believed to be contained in natural gelatin for photographic use.

Certain kinds of gold salts such as aurous thiocyanate also possess a chemical sensitization effect, and the technique of utilizing this effect is well known in the art as "gold sensitization."

It is desired to further increase a sensitivity or speed of photographic silver halide emulsion. A heterocyclic compound having as a basic core the following formula:



has thus been proposed as a sensitizer in U.S. Pat. No. 3,656,955 issued to Ushimaru et al., which is characterized in the presence of five sulfur atoms in the ring (hereafter referred to as a "5-sulfur containing compound"). However, since the 5-sulfur containing heterocyclic ring is unstable, the 5-sulfur containing compound yields more readily a reactive sulfur atom which is inclined to impede proper sensitization. The inclination of the 5-sulfur containing compound to react rapidly with the silver and produce uneven or irregular sensitization calls for special handling of the 5-sulfur containing materials such as the use of diluted solutions, rapid stirring, etc., in the preparation of photographic emulsions. In addition, the 5-sulfur containing compound tends to form an undesired high level of fogging upon storage. The sufficiently high sensitivity without accompanying fog formation is not achieved with those known compounds.

**SUMMARY OF THE INVENTION**

We have discovered that the compounds of the general formula:



wherein R<sub>1</sub> and R<sub>2</sub>, and R<sub>3</sub> and R<sub>4</sub> individually represent hydrogen atoms or alkyl or aralkyl groups or, in combination, cycloalkyl groups, are very useful as sulfur sensitizers for any type of light sensitive silver halide photographic emulsions e.g., silver chloride emulsions, silver bromide emulsions, silver iodide emulsions and composite silver halide emulsions, irrespective of water washing or the lack of water washing and have thus accomplished the object of the present invention, i.e., to enhance the photographic sensitivity of light sensitive silver halide photographic emulsions, with little or no increase in fogging.

The feature of the compounds of our invention which may be referred to as a "4-sulfur containing compound" resides in the hetero ring of the formula:



Thus, the substituents of carbon atoms should not be limited to those mentioned. Any group which does not affect the sensitizing effect of our compound can be attached to the carbon atoms. Our compounds are characterized by this structural arrangement and also by the sensitivity effect which results from this structure. This is, the novel compound of the present invention has moderate reactivity with silver halide in a heterogeneous system as compared to the 5-sulfur containing compound of Ushimaru et al., which serves as uniform sensitization of silver halide which does not cause fog. Further, the 4-sulfur containing compound requires no special care in the preparation of photographic emulsions due to appropriate reactivity with silver halide, whereas the 5-sulfur containing compound must carefully be treated in the preparation of photographic emulsions not so as to give rise to undesirable local reaction with silver halide.

**BRIEF DESCRIPTION OF THE ACCOMPANYING  
DRAWINGS**

FIG. 1 shows a device for potentiometric titration.

FIG. 2 and FIG. 3 are a graphical representation of the molar ratio of silver nitrate to the sensitizer at varying potential levels, in which a sensitizer of this invention was compared with a similar sensitizer but having five sulfur atoms in the heterocyclic ring, as described hereinafter in a comparative example.

**DETAILED DESCRIPTION OF THE INVENTION**

The chemical sensitizers represented by the above general formula can be exemplified by the following compounds, but the chemical sensitizers for use in the practice of the present invention are not restricted thereto.

65  
Compound 1





The optimum amount of the sulfur sensitizer of the above general formula to be added depends on the compound chosen, the silver halide used, the particle size of the silver halide, the temperature and time of ripening and the pH and pAg of the silver halide emulsion, though, in general, the sensitizer compound may be used in the amount within the range of 0.01 mg to 100 mg per mole of silver halide. The smaller particle size, the lower temperature and the shorter time of ripening and the lower pH and higher pAg, the much more amount is requested. When the sensitizer compound is used in combination with another sensitizer, or sensitizers outside the scope of the invention, the amount may be smaller than the lower limit of the above range and, for the case where the compound is used in combination with an antifogging agent, it may be used in a larger amount.

The sulfur sensitizer of the present invention may be used in combination with a reductive sensitizer such as, e.g., stannous salts or thiourea dioxide, with gold-, platinum- and palladium salts such as, e.g., aurous thiocyanate, or with sulfur containing compounds such as, e.g., sodium thiosulfate and thiourea derivatives. In addition, it may be combined with a poly(oxyalkylene) compound of a molecular weight of at least 300 or an onium compound used. Examples of oniums are pyridinium, sulfonium, etc.

The sulfur containing compound of the above general formula in accordance with the present invention may be used not only in spectral sensitization but also in non-spectral sensitization and may be applied to monochromatic photographic emulsions, color photographic emulsions, X-ray photographic emulsions and graphic photographic emulsions.

The sensitizer of the present invention has no adverse effect on stabilizers, antifogging agents, film hardners,

35 color developers, coating aids and other conventional emulsion additives, and these materials may be added in a manner known to the art.

40 While the sulfur sensitizer of the above general formula is useful especially for sensitization of silver halide photographic emulsions prepared from inactive gelatin, it may also be used for sensitization of silver halide photographic emulsions in which at least a portion of the protective colloid is a photographically active gelatin or other hydrophilic colloid, such as polyvinyl alcohol, polyvinyl pyrrolidone and other water soluble synthetic resins well known in the art.

45 The sulfur sensitizer of the present invention has the characteristic that its sensitizing effect is especially enhanced in combination with a thiosulfate compound. The amount of thiosulfate compounds is not critical. Preferably 0.01 to 10 mole per mole of our S-containing compound.

50 Among the compounds represented by the above general formula, Compound 1 can be synthesized by the process disclosed in Chem. Ber. 98, 1454 (1965), Compounds 2 and 3 can be synthesized in accordance with the disclosure in Angew. Chem. 70,682 (1958), Compounds 4 and 5 in accord with Acta. Chem. Scand. 13,1031 (1959) and Compound 6 in accord with Acta. Chem. Scand. 12,890 (1958).

55 The present invention will now be illustrated in greater detail by the following examples.

#### EXAMPLE 1

Prior to beginning the chemical ripening of a high sensitivity, neutral process gelatino-silver iodobromide emulsion (AgI 5.0 mol%, AgBr 95.0 mol %), the emulsion was divided, in equal parts, into 5 specimens (Specimens A to E). To Specimens C to E were added methanolic solutions of Compounds 1, 2 and 3, respec-

tively, and to Specimen B was added natural active gelatin. No addition was made to Specimen A. To each of the specimens there was then added an aqueous solution of 7.5 mg of chloroauric acid, 0.01 wt percent of aqueous solution was used, as a gold sensitizer and 150 mg of potassium thiocyanate per mole of silver halide. The emulsions were then subjected to chemical ripening at 50°C for 60 minutes with stirring. The chloroauric acid used was the tetrahydrate. To 1 Kg of the chemically ripened emulsion there was added 30 mg of 3,3-diethyl-9-methylthiacarbocyanine bromide, 450 mg of chrome alum and 120 mg of saponin, and the emulsion was applied onto a cellulose triacetate film base and dried to provide a sensitive material (coating thickness: 14 microns). The material thus obtained was exposed one-fiftieth of a second with an optical wedge to a light source at a color temperature of 5,400°K, developed at 20°C for 10 minutes using a developer of the following formulation, fixed, washed with water and dried, and subjected to sensitometric analysis to obtain the data listed in Table 1.

| Developer                         |         |
|-----------------------------------|---------|
| N-methyl-para-aminophenol sulfate | 2.0 g   |
| Anhydrous sodium sulfite          | 100.0 g |
| Hydroquinone                      | 5.0 g   |
| Borax                             | 2.0 g   |
| Water to make 1000 ml of solution |         |

Table 1

| Specimen | Sulfur sensitizer | Amounts added/ mole of AgX | Relative Sensitivity | Gamma | Fog  |
|----------|-------------------|----------------------------|----------------------|-------|------|
| A        | —                 | —                          | 100                  | 0.43  | 0.04 |
| B        | Active gelatin    | 10 g                       | 1100                 | 0.89  | 0.12 |
| C        | Compound 1        | 70 mg                      | 1120                 | 0.92  | 0.08 |
| D        | Compound 2        | 80 mg                      | 1240                 | 0.92  | 0.09 |
| E        | Compound 3        | 75 mg                      | 1240                 | 0.91  | 0.09 |

As is evident from the Table 1, marked sensitization effects were noticed for Specimens C, D and E. When the compound of the present invention was used the higher sensitivity without increasing fog formation was obtained in comparison with known active gelatin.

## EXAMPLE 2

Prior to beginning chemical ripening of a fine grain positive, neutral process gelatino-silver chlorobromide emulsion (AgBr 58.0 mol %, AgCl 42.0 mol %), the emulsion was divided into three equal parts (Specimens A to C). A methanolic solution of Compound 4 was added to Specimen C, a natural sensitized gelatin to Specimen B (in amounts as listed in Table 2) and nothing was added to Specimen A. The three emulsions were then aged at 52°C for 50 minutes and, thereafter, there was added thereto, per 1 Kg of each emulsion 300 mg of 4-hydroxy-6-methyl-1,3,3a,7-tetrazaindene, 450 mg of chrome alum and 120 mg of saponin. Each emulsion was then applied onto a cellulose triacetate base and dried to obtain a sensitive material (coating thickness: 12 microns). The materials were then exposed one-twentieth of a second with an optical wedge to a light source at a color temperature of 2,660°K, developed at 20°C for 10 minutes using a developer of the following formulation, fixed, washed with water and dried, and subjected to sensitometric analysis to obtain the data listed in Table 2, which data indicates a marked sensitizing effect for the sensitizer of the present invention.

oped at 20°C for 4 minutes with a developer of the following formulation, fixed, washed with water, dried and then subjected to a sensitometric analysis to obtain the data summarized in Table 2, which data indicates a marked sensitizing effect for the sensitizer of the present invention.

## Developer

|                                   |        |
|-----------------------------------|--------|
| N-methyl-para-aminophenol sulfate | 1.4 g  |
| Potassium bisulfite               | 8.0 g  |
| Hydroquinone                      | 6.0 g  |
| Sodium carbonate monohydrate      | 22.5 g |
| Citric acid                       | 0.7 g  |
| Potassium bromide                 | 0.9 g  |
| Water to make 1000 ml of solution |        |

Table 2

| Specimen | Sulfur sensitizer          | Amount added/ mole of AgX | Relative Sensitivity | Gamma | Fog  |
|----------|----------------------------|---------------------------|----------------------|-------|------|
| A        | —                          | —                         | 100                  | 1.20  | 0.04 |
| B        | Natural sensitized gelatin | 14 g                      | 1050                 | 2.61  | 0.05 |
| C        | Compound 4                 | 100 mg                    | 1120                 | 2.68  | 0.05 |

## EXAMPLE 3

Prior to beginning of chemical ripening of a coupler in developer type reversal color, high sensitivity, neutral process gelatino-silver iodobromide emulsion (silver iodide 5.0 mol percent, silver bromide 95.0 mol percent), the emulsion was divided into equal five parts (Specimens A to E). There was added to Specimen B a natural sensitized gelatin in amounts as listed in Table 3, and nothing was added to Specimen A. The five emulsions then had added thereto, per 1 mole of silver halide, 7.5 mg of chloroauric acid tetrahydrate and 150 mg of sodium thiocyanate in solution in water, and the emulsions were subjected to chemical ageing at 50°C for 70 minutes with stirring. Each emulsion then had added thereto, per 1 Kg of emulsion, 30 mg of 1,3-diethyl-5'-methoxy-6-methylselena-2-cyanine iodide, 450 mg of chrome alum and 120 mg of saponin, was applied to a cellulose triacetate base and dried to obtain a sensitive material (coating thickness 8 microns). The material thus obtained was exposed one-twentieth of a second with an optical wedge to a light source at a color temperature of 5,400°K, developed at 27°C for 3 minutes and 30 seconds with a developer of the following formulation, fixed, washed with water, dried, and subjected to sensitometric analysis to obtain the data summarized in Table 3, which data indicates a remarkable sensitizing effect for the sulfur sensitizer of the present invention.

## Developer

|                                        |        |
|----------------------------------------|--------|
| N-methyl-para-aminophenol sulfate      | 1.0 g  |
| Anhydrous sodium sulfite               | 60.0 g |
| Hydroquinone                           | 10.0 g |
| Potassium bromide                      | 5.0 g  |
| Potassium thiocyanate                  | 1.5 g  |
| 0.1% aqueous potassium iodide solution | 5.0 ml |
| Sodium hydroxide                       | 2.0 g  |
| Water to make 1000 ml of solution      |        |

Table 3

| Specimen | Sulfur sensitizer          | Amounts added mole of AgX | Relative sensitivity | Gamma | Fog  |
|----------|----------------------------|---------------------------|----------------------|-------|------|
| A        | —                          | —                         | 100                  | 0.46  | 0.07 |
| B        | Natural sensitized gelatin | 10 g                      | 1020                 | 0.82  | 0.16 |
| C        | Compound 5                 | 55 mg                     | 1020                 | 0.87  | 0.13 |
| D        | Compound 5                 | 60 mg                     | 1240                 | 0.89  | 0.16 |
| E        | Compound 5                 | 65 mg                     | 1100                 | 0.86  | 0.13 |

## EXAMPLE 4

Prior to beginning of chemical ripening of an ammonia process gelatin-silver iodobromide emulsion (AgI 1.5 mol%, AgBr 98.5 mol%), the emulsion was divided into three equal parts (Specimens A to C), and to Specimens B and C there was added, respectively, Compounds 1 and 2, both in methanolic solution, in amounts as listed in the Table 4. To Specimens A was added, per mole of silver halide, 4.7 mg of sodium thiosulfate five pentahydrate and 1.2 mg of sodium dithiosulfatoauroate dihydrate  $\text{Na}_3\text{Au}(\text{S}_2\text{O}_3)_2 \cdot 2\text{H}_2\text{O}$  in aqueous solution, while to Specimen B these materials were added in an amount, per mole of silver halide, respectively, of 4.7 mg and  $3.2 \times 10^{-2}$ , while to Specimen C there was added, per mole of silver halide, 1.2 mg of sodium dithiosulfatoauroate dihydrate alone. The emulsions were then subjected to chemical ripening at 50°C for 70 minutes. The emulsion was then applied to a poly(ethylene terephthalate) film base and dried to obtain a sensitive material (coating thickness: 8 microns). The material thus obtained was exposed one-twentieth of a second with an optical wedge to a light source at a color temperature of 5,400°K, developed at 20°C for 4 minutes with a developer of the following formulation, and subjected, after fixing, washing with water and drying, to sensitometric analysis to obtain the data summarized in Table 4.

that obtained in the case of Specimen A where the sulfur sensitizer was used alone. The marked effect shown in Examples 1 to 4 was, of course, Compounds 3 and 4.

## EXAMPLE 5

Prior to beginning of chemical ripening of a negative color, high sensitivity, neutral process gelatin-silver iodobromide emulsion (AgI 7.0 mol %, AgBr 93.0 mol %), the emulsion was divided into four equal parts (Specimens A to D).

However, it should be noted that our compound may be added to silver halide emulsion not only prior to the chemical ripening but also during the chemical ripening. In short, the chemical ripening may be conducted in the presence of our compound.

There was added, in amounts as listed in Table 5, a natural sensitized gelatin to the Specimen B, a natural sensitized gelatin and Compound 2 to Specimen C and Compound 2 to the Specimen D. Nothing was added to Compound A. To the four emulsions, there was then added, per mole of silver halide, 5.0 mg of chloroauric acid tetrahydrate and 5.0 mg of potassium thiocyanate in aqueous solution, and the emulsions subjected to chemical ageing at 60°C for 50 minutes with stirring. To 1 Kg of the emulsions there was added 180 mg of 3,3',9-triethyl-5,5'-dichlorothiacarbocyanine bromide, 300 mg of 4-hydroxy-6-methyl-1,3,3',7-tetrazaindene, 5 g of cyan coupler and 5 g of colored cyan coupler each described in Example of British Pat. No. 1,146,368, 450 mg of chrome alum and 120 mg of saponin were also added and the emulsions applied to a cellulose triacetate film base and dried to obtain a red sensitive color photographic light sensitive material (coating thickness: 5 microns).

The color sensitive material was exposed one one-hundredth second, at a color temperature of 5,400°K through an optical wedge to a red-colored light and subjected to color development in a conventional manner with a color developer of the following formulation.

| Developer                         |        |
|-----------------------------------|--------|
| N-methyl-para-aminophenol sulfate | 4.0 g  |
| Anhydrous sodium sulfite          | 60.0 g |
| Hydroquinone                      | 10.0 g |
| Sodium carbonate monohydrate      | 53.0 g |
| Sodium bromide                    | 3.0 g  |
| Water to make 1000 ml of solution |        |

| Color developer                                     |        |
|-----------------------------------------------------|--------|
| N,N-diethyl-para-aminophenol sulfate                | 2.0 g  |
| Sodium sulfate                                      | 2.0 g  |
| Sodium carbonate monohydrate                        | 50.0 g |
| Hydroxylamine hydrochloride                         | 1.5 g  |
| Potassium bromide                                   | 1.0 g  |
| Water to make 1000 ml of solution (pH = 10.8 ± 1.0) |        |

Table 4

| Specimen | Sulfur sensitizer                                                                                                                                                                | Amounts added/ mole of AgX               | Relative sensitivity | Gamma | Fog  |
|----------|----------------------------------------------------------------------------------------------------------------------------------------------------------------------------------|------------------------------------------|----------------------|-------|------|
| A        | $\text{Na}_2\text{S}_2\text{O}_3 \cdot 5\text{H}_2\text{O}$<br>$\text{Na}_3\text{Au}(\text{S}_2\text{O}_3)_2 \cdot 2\text{H}_2\text{O}$                                          | 4.7 mg<br>1.2 mg                         | 100                  | 1.95  | 0.12 |
| B        | $\text{Na}_2\text{S}_2\text{O}_3 \cdot 5\text{H}_2\text{O}$                                                                                                                      | 4.7 mg                                   | 121                  | 1.96  | 0.12 |
| C        | $\text{Na}_3\text{Au}(\text{S}_2\text{O}_3)_2 \cdot 2\text{H}_2\text{O}$<br>Compound 1<br>$\text{Na}_3\text{Au}(\text{S}_2\text{O}_3)_2 \cdot 2\text{H}_2\text{O}$<br>Compound 2 | $3.2 \times 10^{-2}$ mg<br>2 mg<br>15 mg | 115                  | 1.93  | 0.13 |

In Specimens B and C, where a sulfur sensitizer of the present invention was used in combination with sodium thiosulfate and/or sodium dithiosulfatoauroate, the sensitizing effect obtained was remarkably greater than

The material was then bleached and fixed with bleaching and fixing solutions of the following formulations to eliminate undeveloped silver halides and reduced silver formed in development.

| Bleaching solution                                  |       |
|-----------------------------------------------------|-------|
| Ferricyanide                                        | 100 g |
| Potassium bromide                                   | 20 g  |
| Water to make 1000 ml of solution<br>(pH 6.9 ± 0.3) |       |
| Fixing solution                                     |       |
| Hypo                                                | 200 g |
| Sodium sulfite                                      | 20 g  |
| Acetic acid (28°C)                                  | 4.5 g |
| Boric acid                                          | 7.5 g |
| Potash alum                                         | 20 g  |
| Water to make 1000 ml of solution<br>(pH 4.5 ± 0.2) |       |

Thus, there was obtained on each Sample a red positive image formed by the color coupler remaining in the film and a developed cyan negative image.

The color images obtained in Specimens A to D were subjected to sensitometric analysis to obtain the data summarized in Table 5, which indicates the remarkable sensitizing effect of the sulfur sensitizer of the present invention.

On the other hand, in the case of the 4-sulfur containing compound, the potential curve is almost the same as that of a blank, i.e., buffer solution. This means that no appreciable reaction of the 4-sulfur containing compound with silver ions occurred during the titration (titration rate for both samples: 5 minutes/one equivalent). Further, the solution containing the 4-sulfur containing compound of the present invention was allowed to stand. The gradual formation of silver sulfide was observed.

The gradual formation of silver sulfide as in the present invention is important for uniform sensitization of the emulsion. This is because chemical sensitization with a sulfur sensitizer proceeds in a heterogenous system, that is, the released sulfur ions from the sulfur sensitizer react with halide in the form of a heterogenous dispersion thereof to form silver sulfide, which silver sulfide is deposited on the surface of silver halide to sensitize silver halide. Accordingly, excessive reactivity of the sulfur sensitizer with silver halide causes uneven deposition of silver sulfide on the surface of silver halide.

Table 5

| Specimen | Sulfur sensitizer          | Amounts added/<br>Mole of AgX | Relative sensitivity | Gamma | Fog  |
|----------|----------------------------|-------------------------------|----------------------|-------|------|
| A        | —                          | —                             | 100                  | 0.33  | 0.03 |
| B        | Natural sensitized gelatin | 10 g                          | 1200                 | 0.63  | 0.08 |
| C        | Natural sensitized gelatin | 10 g                          | 1350                 | 0.67  | 0.07 |
| D        | Compound 2                 | 50 g                          | 1500                 | 0.65  | 0.07 |
|          | Compound 2                 | 75 mg                         |                      |       |      |

#### COMPARATIVE EXAMPLE

1. Solutions of Compound 2 of the present invention and Compound 1 of U.S. Pat. No. 3,656,955 Ushimaru et al. (each in methanol) were prepared (concentration 1/1000 mole/l) and maintained at 50°C in a constant temperature bath.

Variations in potential of these samples were measured by a potentiometric titration using a device as shown in FIG. 1, that is, a 0.1 N aqueous silver nitrate solution was added dropwise to the solutions which were maintained at 50°C, using an automatic titration buret to record the variations of potential on an automatic recorder.

The results are shown in FIGS. 2 and 3 in which the vertical axis shows electrical potential and the horizontal axis shows the molar ratio of silver nitrate to the 4-sulfur containing compound on the 5-sulfur containing compound. The change in potential as will be understood by one skilled in the art, corresponds to the change of the concentration of free silver ions. From these figures it can easily be seen that for the 5-sulfur containing compound of Ushimaru et al. the potential was small at low concentrations of silver nitrate at pH 7 and pH 9. This means that the compound of Ushimaru et al immediately reacted with silver nitrate (removed free silver ions) to form silver sulfide.

ide due to local occurrence of the formation of silver sulfide.

From the above data, it can thus be seen that special care is not required in the present invention because of the moderate and appropriate reactivity of the 4-sulfur containing compound, while the reactivity of the 5-sulfur containing compound with silver ions is so drastic that special care such as adding as a diluted solution, rapid stirring, etc., is required in the preparation of photographic emulsions.

2. This experimentation was conducted to compare the photographic effects of the 5-sulfur containing compound of U.S. Pat. No. 3,656,955 Ushimaru et al. with the 4-sulfur containing compound of the present invention.

The experimentation was conducted using an emulsion obtained in accordance with the method described in Example 4 of the present specification. To separate but identical emulsions each of natural sensitized gelatin, Compound 1 of Ushimaru et al. and Compound 2 of the invention were added, respectively. The emulsions were then exposed as in Example 4 immediately after coating or after being subjected to an incubation test for 3 days at 50°C under the relative humidities listed in Table 6 to determine the amount of fog which would occur.

Table 6

| Sensitizer                      | Amount added/<br>mole of AgX | Relative<br>Sensitiv-<br>ity | Fog                       |      | After 3 days<br>50°C 30% RH | After 3 days<br>50°C 80% RH |
|---------------------------------|------------------------------|------------------------------|---------------------------|------|-----------------------------|-----------------------------|
|                                 |                              |                              | Immediately After Coating | **   |                             |                             |
| A. Natural sensitized gelatin   | 15 g                         | 100                          | 0.05                      | 0.26 | 0.29                        |                             |
| B. Compound 1 of Ushimaru et al | 5 mg                         | 115                          | 0.05                      | 0.28 | 0.28                        |                             |
| C. Compound 2 of the invention  | 30 mg                        | 115                          | 0.05                      | 0.19 | 0.20                        |                             |

TABLE 6—Continued

| Sensitizer | Amount added/<br>mole of AgX | Relative<br>Sensitiv-<br>ity | Fog<br>Immediately After Coating | **<br>After 3 days<br>50°C 30% RH | **<br>After 3 days<br>50°C 80% RH |
|------------|------------------------------|------------------------------|----------------------------------|-----------------------------------|-----------------------------------|
|------------|------------------------------|------------------------------|----------------------------------|-----------------------------------|-----------------------------------|

\* The amount of the sensitizers to be added was arranged to gain the same value of the relative sensitivity, that is, Compound 2 which had slow reactivity with silver ions as shown in (1) above was used in a six times amount as compared to Compound 1 of the prior art. As a decrease in fog is often more significant than an increase in sensitivity in the art, the greatest chance of fairly comparing both compounds would be given by leveling the relative sensitivity thereof.

\*\* The conditions were set out under careful consideration of the practical use in the changeable climate in Japan and are believed to be representative of in-use condition under high temperatures at low humidity and at high humidity.

As is shown in Table 6, the fog values for the samples 10 are the same immediately after coating but, after incubating the samples for 3 days, Samples A and B show an increase in fog. On the other hand, in Sample C containing the sensitizer of the present invention, the increase in fog is as compared to Samples A and B. In 15 more detail, the increase in fog of Sample C was merely 0.14 after standing for 3 days at 50°C under the relative humidity of 30 percent and 0.15 after standing for 3 days at 50°C under the relative humidity of 80 percent, whereas, in Sample B, the increase in fog was 0.23 under both conditions. If the increase in fog,  $\Delta$ fog, exceeds 2.0 a photographic emulsion will be unfit for the practical use even if it has a considerably high sensitivity.

From the results presented in the comparative study 25 (1) and (2), it can be seen that the 5-sulfur containing compound of the prior art harmed the photographic properties, i.e., increased fog during storage thereof, and that such a material cannot be equated to the 4-sulfur containing compounds of the present invention.

While the invention has been described in detail and with reference to specific embodiments thereof, it will be apparent to one skilled in the art that various changes and modifications can be made therein without departing from the spirit and scope thereof.

What is claimed is:

1. A photosensitive silver halide emulsion containing 25 at least one compound of the formula:



wherein R<sub>1</sub>, R<sub>2</sub>, R<sub>3</sub> and R<sub>4</sub> each individually may be a hydrogen or a lower alkyl group.

R<sub>1</sub> and R<sub>2</sub> may combine with the bonded carbon of the sulfur containing ring and with themselves to form a cycloalkyl group containing up to six carbon

R<sub>3</sub> and R<sub>4</sub> may combine with the bonded carbon of the sulfur containing ring and with themselves to form a cycloalkyl group containing up to six carbon atoms, including the carbon of the sulfur containing ring,

said compound being present in said photosensitive silver halide emulsion in an amount of from about 0.01 to 100 mg per mole of silver halide.

2. The photosensitive silver halide emulsion of claim 1 wherein said compound is



30 3. The photosensitive silver halide emulsion of claim 1 wherein said compound is



35 40 4. The photosensitive silver halide emulsion of claim 1 wherein said compound is



45 50 5. The photosensitive silver halide emulsion of claim 1 wherein said compound is



atoms, including the carbon atom of the sulfur containing ring, and

6. The photosensitive silver halide emulsion of claim 1 wherein said compound is



7. The photosensitive silver halide emulsion of claim 1 wherein said compound is



8. The photosensitive silver halide emulsion of claim 1 further containing from about 0.01 to 10 moles per mole of said compound of a thiosulfate compound.

9. The photosensitive silver halide emulsion of claim 2 further containing from about 0.01 to 10 moles per mole of said compound of a thiosulfate compound.

10. The photosensitive silver halide emulsion of claim 3 further containing from about 0.01 to 10 moles per mole of said compound of a thiosulfate compound.

11. The photosensitive silver halide emulsion of claim 4 further containing from about 0.01 to 10 moles per mole of said compound of a thiosulfate compound.

12. The photosensitive silver halide emulsion of claim 5 further containing from about 0.01 to 10 moles per mole of said compound of a thiosulfate compound.

13. The photosensitive silver halide emulsion of claim 6 further containing from about 0.01 to 10 moles per mole of said compound of a thiosulfate compound.

14. The photosensitive silver halide emulsion of claim 7 further containing from about 0.01 to 10 moles per mole of said compound of a thiosulfate compound.

15. The pressure sensitive silver halide emulsion of claim 1 wherein said compound is used in combination

with another sensitizer and the amount of said compound is up to 100 mg per mole of silver halide.

16. The photosensitive silver halide emulsion of claim 1 wherein said compound is used in combination with an antifogging agent and the amount of said compound is above 0.01 mg per mole of silver halide.

17. The photosensitive silver halide emulsion of claim 15 further containing from about 0.01 to 10 moles per mole of said compound of a thiosulfate compound.

18. The photosensitive silver halide emulsion of claim 16 further containing from about 0.01 to 10 moles per mole of said compound of a thiosulfate compound.

19. The photosensitive silver halide emulsion of claim 1 wherein said cycloalkyl group is one selected from the group consisting of a cyclobutyl group, a cyclopentyl group and a cyclohexyl group.

20. The photosensitive silver halide emulsion of claim 8 wherein said thiosulfate compound is one selected from the group consisting of sodium thiosulfate, aurous thiosulfate salt, thiourea derivatives and mixtures thereof.

\* \* \* \* \*